

## UNITED STATES PATENT OFFICE.

GEORGE W. HALLOCK, OF BLOOMFIELD, NEW JERSEY, ASSIGNOR TO WESTINGHOUSE LAMP COMPANY, A CORPORATION OF PENNSYLVANIA.

## ALLOY BASE FOR OXIDE-COATED CATHODES.

No Drawing.

Application filed October 27, 1927. Serial No. 229,276.

This invention relates to electron-emitting cathodes of the oxide coated type, such as are used in thermionic discharge devices, and more particularly to an electrically conductive core or base for such cathodes.

Heretofore in the manufacture of oxide coated cathodes it has been the usual practice to employ a core of nickel or platinum-iridium alloy. Nickel has very largely superseded the use of platinum-iridium, due to the excessive expense of the platinum. Nickel has the disadvantage, however, in that its specific resistance is such that the voltage-ampere characteristics required for the large size filaments cannot be readily obtained without reducing the thickness of the core to such an extent that it is mechanically weak or, if proportioned for proper tensile strength, causing it to operate at an excessively high temperature, either of which result in short life.

For instance, with large sizes of ribbon, in order to obtain the required voltage and amperage characteristics, and the requisite surface area to maintain the proper operating temperature, it is necessary to roll the core into a ribbon of considerable width and of an extreme thinness, below 1 mil. Great difficulty is involved in uniformly rolling the material to this degree of thinness and the edges become frayed and feathered so that the ribbon is easily torn and does not have sufficient strength to withstand the strain required to maintain it taut on the mount. The ribbon is, therefore, made thicker and narrower than theoretically required in order to increase the tensile strength but due to the decrease in heat radiating surface thus occasioned, the cathode operates at an excessively high temperature. This high filament temperature results in bombardment of the cathode by back emission from the grid or plate, caused by the thermionically active coating on the cathode being thrown off at the high operating temperature thereof and depositing on the grid, and the heating of the grid, to an electron emitting temperature by heat radiated from the overly heated cathode. This back bombardment rapidly destroys the filament.

Difficulty has also been experienced in the smaller size filaments when employing nickel cores, in causing the oxide coating to adhere, since in order to obtain the required voltage-ampere characteristics, it is necessary to go to the other extreme, and make the ribbon

narrow and thick, rather than broad and thin. The oxide coating does not adhere as readily to the narrow ribbon as it does to the broader surface.

The hot strength of nickel is low, moreover, which contributes materially to the failures due to breakage of both the smaller sized and the extremely thin nickel ribbons.

One of the objects of the present invention is to overcome the above mentioned difficulties and to produce a metal core for an oxide coated cathode which will have the proper specific resistance to enable the required voltage-ampere characteristics to be readily obtained at the proper operating temperature and which will be strong and rugged.

A further object is to provide an electrically conductive core which will have a high tensile strength while hot.

A still further object is to provide a thermionically active cathode which will have a large electron-emitting surface area for a given voltage and current requirement.

Other objects and advantages will herein-after appear.

In accordance with my invention, I employ as the electrically conductive core an alloy of nickel with another metal which will alter its specific resistance so as to enable the proper physical and electrical characteristics to be obtained. For the large size filament, I employ an alloy having a higher specific resistance than pure nickel, whereas, for the smaller size filaments, I employ an alloy having a lower specific resistance than nickel.

Thus, for instance, in producing cores for cathodes of large size, that is, having a filament weight corresponding to an 8 mil wire, in order to meet the voltage and amperage requirements which have become standardized in the radio industry and maintain proper operating temperature of the filament, it would be necessary to flatten an 8 mil nickel wire to a width of about 40 mil and a thickness of less than 1 mil. This is not practical, however, due to the low tensile strength of nickel, and the extreme fragility of a ribbon of this thinness. I have found, however, that certain alloys, such as an alloy of silicon and nickel or manganese and nickel in the proper proportions have a higher specific resistance than pure nickel and, therefore, that it is possible to employ a thicker ribbon of substantially the same width and which will, therefore, have increased tensile strength in

proportion to the increase in size. Silicon-nickel and manganese-nickel have greater hot strength than pure nickel moreover so that the strength of the filament is still further increased.

For the large size wires, silicon-nickel is preferred since its change in specific resistance for various percentages is very slight. An alloy containing about 3% of silicon I have found very satisfactory, but the percentage may run from 2 to 6% without materially altering the electrical conductivity of the metal. This is advantageous since it eliminates the necessity of maintaining exact proportions in the fabrication of the wire. Manganese-nickel with a manganese content of 4% is also satisfactory for large filaments, but the proper percentage of manganese must be more carefully maintained, since the conductivity varies considerably with the change in manganese content.

Pure nickel ribbon of a weight corresponding to a 6 or 8 mil wire has a specific resistance of about 5.35 ohms per sq. cm., whereas, the alloys which I prefer for filaments of this weight have a specific resistance of about 6.

For small size wires, it is desirable that the specific resistance of the metal core be lower than that afforded by pure nickel in order to meet the standard requirements. In the case of pure nickel, as the weight of the filament is decreased, for use in tubes of smaller output, the thickness of the filamentary core increases and the width decreases so that for the smallest size filaments the thickness approaches the width. When these conditions are obtained, difficulty is experienced in causing the oxide coating to properly adhere to the small flat surface presented by the narrow ribbon. In such case, I have found that an alloy such as an alloy of manganese and nickel containing about 2% of manganese, which has a lower specific resistance than nickel, may be shaped into a relatively broad and thin ribbon while maintaining the required voltage and amperage conditions and the proper operating temperature. This broad ribbon presents a more extensive surface to which the oxide coating will adhere more tenaciously. It also increases the electron emitting area of the cathode and thereby enhances the electron emitting property of the coated cathode. In these small size wires the increased tensile strength afforded by the alloy core increases very materially the life of the device in which it is employed.

I have further found that the silicon or manganese-nickel alloy cores are not as susceptible to variations in their specific resistances by internal changes in the core as is nickel. In the case of pure nickel, the conductivity varies according to the particular

heat treatment and mechanical working to which it is subjected.

It is the practice in the manufacture of electron discharge devices employing oxide coated cathodes to subject the filament in the completely assembled tube during the exhaust treatment to a high temperature flash while the other electrodes are being degassed in order to prevent absorption by the cathode of gas liberated from the other electrodes. This high temperature flash is much in excess of the normal operating temperature of the cathode and changes the electrical conductivity of the wire, probably due to a change in the internal construction of the metal core. Therefore, in designing nickel cores for oxide coated cathodes, it is necessary to take into consideration the change in conductivity effected by this high temperature treatment. Since this treatment is not uniform in all tubes, the electrical conductivity of filament cores of the same size is not uniform and this non-uniformity has caused considerable difficulty.

In the case of silicon-nickel or manganese-nickel alloy, I have found that this high temperature treatment does not materially vary the electrical conductivity and much greater uniformity in the electrical characteristics of the cathodes is obtained and the design of the core considerably simplified.

One of the difficulties, which has been mentioned before, when employing large oxide coated cathodes with nickel cores has been the high temperature at which the cathodes necessarily operate by virtue of the fact that they must be made thicker and narrower than they should be theoretically, in order to impart the necessary mechanical strength thereto. The proper operating temperature, particularly in tubes having a large power output, must be carefully observed, since if the temperature is too high the oxide coating sputters or otherwise becomes transferred over to the other electrodes. These other electrodes become highly heated by radiation from the cathode so that they themselves become thermionically active and the electrons emitted therefrom bombard the filament and rapidly disintegrate the same so that it quickly burns out. Due to the greater specific resistance of silicon-nickel or manganese-nickel when employed as a core for filament of large size, the heat radiating area is increased for the same voltage and current conditions and consequently the filament operates at a lower temperature, whereby the difficulties due to back emission are eliminated.

It should be understood that while silicon and manganese have been specified as the particular alloying ingredients in definite proportions, that the invention is not limited to these specific details, but equivalent metals may be employed and other proportions, de-

pending upon the particular conditions which it is necessary to attain.

What is claimed is:

1. An electrically conductive core for a thermionically active cathode comprising an alloy of nickel and silicon.
2. An electron-emitting cathode comprising an alloy of nickel and silicon and a coating thereon of thermionically active material.
3. A metal core for an electron-emitting

cathode of the oxide coated type composed of an alloy of nickel and about 3% of silicon.

4. An electron-emitting cathode comprising a core composed of an alloy of a metal of the group containing nickel and up to 6% of silicon.

In testimony whereof, I have hereunto subscribed my name this 26th day of October, 1927.

GEORGE W. HALLOCK.